

## 1

3,475,174

### N,N DIALKYL N' ACYL-DIAMINOCARBOXYLIC ACID COATING COMPOSITIONS

Shui Sato, Hachioji-shi, Tokyo, Eiichi Sakamoto, Hannō-shi, and Setsuji Sakurai, Fujisawa-shi, Japan, assignors to Konishiroku Photo Industry Co., Ltd., Tokyo, Japan, and Ajinomoto Co., Inc., Tokyo, Japan  
No Drawing. Filed Mar. 23, 1966, Ser. No. 536,628  
Claims priority, application Japan, Mar. 29, 1965,

40/17,767

Int. Cl. G03c 1/02; C09d 3/04  
U.S. Cl. 96—94

7 Claims

### ABSTRACT OF THE DISCLOSURE

Novel compounds and photographic coating compositions comprising same. The compounds are of the formula:



wherein either X or Y is a lower dialkyl amino group of the formula



wherein R<sub>1</sub> and R<sub>2</sub> are lower alkyl groups and the other of X and Y is an amide group of the formula —NHR<sub>3</sub> wherein R<sub>3</sub> is an acyl group of 6 to 18 carbon atoms; M is hydrogen or a lower alkyl group and n is an integer from 2 to 4 inclusive.

This invention relates to N,N-dialkyl-N'-acyl-diamino-carboxylic acids, their lower alkyl esters and their acid addition salts. In the particular aspect, the present invention is directed to photographic layers containing the above-mentioned compounds as coating aids.

Photographic light-sensitive materials usually have a support and a plurality of layers coated thereon. Among these layers there are included backing layer, subbing layer, light-sensitive emulsion layer, protective or anti-halation layer, filter layer, etc. In the routine work of the art, these layers are formed on the film support by applying a coating liquid (solution, emulsion or dispersion) to the support and then drying the coating. In this case, it is very essential to apply a variety of coating liquids onto the entire surface of the support at uniform thickness. In the prior art, however, unevenness in the coating directions (frequently referred to as "longitudinal unevenness" or "transverse unevenness") and local imperfection of coating (frequently referred to as "comets") or unevenness at the peripheral zone are occasionally observed. In order to prevent such drawbacks, use of a coating aid, e.g. a surface tension depressant for coating liquids, is well known in the art.

Among the known coating aids, saponine is the most common. Because the saponine is a material of the natural origin, however, use of the saponine unavoidably causes an adverse effect on the photographic properties of the resulting film due to the varying quality of said saponine. Alternatively, use of certain synthetic surface active agents also has been proposed. However, the known surface active agents are not fully satisfactory, as they usually have an adverse influence on the photographic properties, e.g. storability under high humidity at high temperature, and show only poor ability to decrease surface tension and contact angle.

Another serious problem encountered in the prior art is undesired formation of static marks in an emulsion

## 2

layer as the result of static electricity induced on film base when dried photographic film is brought into frictional condition. Prevention of the formation of such static marks, as well as improvement in coating uniformity, is highly desirable in the art, but unfortunately it is to be said that such a compound which can provide both effects has never been known.

Now we have found that a compound of the general formula



wherein one of X and Y is a group



(wherein R<sub>1</sub> and R<sub>2</sub> individually mean lower alkyl) and the other is a group —NHR<sub>3</sub> (wherein R<sub>3</sub> is acyl group having 6 to 18 carbon atoms); M is hydrogen or lower alkyl; and n is an integer of 2, 3 or 4, or the salt thereof, is useful as coating aid which permits us to be free from any disadvantages of the prior art coating techniques.

Thus, if the above-indicated compound is used as a coating aid singly or in combination with any other known surface active agent, a film-coating liquid containing said coating aid shows an appreciable decrease in viscosity, thereby to facilitate high speed coating at about 40 m./min., without formation of uneven coating or comets. Not only the formation of uniform coating but also the antistatic effect is provided by the present invention. A particular advantage of the present invention is that the compounds used therein has no little adverse influence on the photographic properties of the film produced. Thus, a coating aid of the present invention can be incorporated, without harmful effect, into not only photographic gelatinous emulsions but also various photographic dispersions which may contain a synthetic polymer (e.g. polyvinyl alcohol) as a binder.

Typical compounds which are usable in the present invention will be illustrated below. However, it should be noted that they are merely illustrative and do not limit the scope of the invention. Effectiveness of these compounds in the photographic application is entirely independent on the optical activity of the said compounds.

| Compound's No. | Chemical Name                                                                                                   | M.P., °C. |
|----------------|-----------------------------------------------------------------------------------------------------------------|-----------|
| 50 I           | N <sup>a</sup> ,N <sup>a</sup> -dimethyl-N <sup>a</sup> -stearoyl-DL-ornithine                                  | 154-156   |
| II             | N <sup>a</sup> ,N <sup>a</sup> -dimethyl-N <sup>a</sup> -myristoyl-DL-ornithine                                 | 120-125   |
| III            | N <sup>a</sup> ,N <sup>a</sup> -dimethyl-N <sup>a</sup> -lauroyl-DL-ornithine                                   | 159-161   |
| IV             | N <sup>a</sup> ,N <sup>a</sup> -dimethyl-N <sup>a</sup> -palmitoyl-DL-lysine                                    | 132-134   |
| V              | N <sup>a</sup> ,N <sup>a</sup> -dimethyl-N <sup>a</sup> -lauroyl-DL-lysine                                      | 162-164   |
| VI             | N <sup>a</sup> ,N <sup>a</sup> -dimethyl-N <sup>a</sup> -caproyl-DL-lysine                                      | 141-146   |
| VII            | N <sup>a</sup> -palmitoyl-N <sup>a</sup> ,N <sup>a</sup> -dimethyl-L-lysine                                     | 123-124.5 |
| VIII           | N <sup>a</sup> -palmitoyl-N <sup>a</sup> ,N <sup>a</sup> -dimethyl-L-lysine methyl ester hydrochloride          | 86-88     |
| IX             | N <sup>a</sup> ,N <sup>a</sup> -dimethyl-N <sup>a</sup> -palmitoyl-DL- $\alpha$ , $\gamma$ -diaminobutyric acid | -----     |
| X              | N <sup>a</sup> ,N <sup>a</sup> -dimethyl-N <sup>a</sup> -oleyl-DL-lysine                                        | 139-143   |
| XI             | N <sup>a</sup> ,N <sup>a</sup> -diethyl-N <sup>a</sup> -lauroyl-DL-ornithine                                    | -----     |
| XII            | N <sup>a</sup> -lauroyl-N <sup>a</sup> ,N <sup>a</sup> -dimethyl-L-lysine methyl ester hydrochloride            | 65-67     |
| XIII           | N <sup>a</sup> ,N <sup>a</sup> -dimethyl-N <sup>a</sup> -lauroyl-DL-ornithine methyl ester (syrup)              | -----     |

These compounds can be easily obtained by converting a diamino-carboxylic acid (e.g. ornithine or lysine) having a di-lower alkyl substituent at either one of N<sup>a</sup>- and N<sup>a</sup>-positions into the copper salt or ester and then reacting the resulted compound, which carboxyl group has been blocked, with an acylating agent donating an acyl group of 6 to 18 carbon atoms, e.g. stearoyl chloride, palmitoyl chloride, etc. For information, typical pro-

cedures for the preparation of certain compounds will be described below:

$N^a,N^a$ -dimethyl- $N^e$ -lauroyl-DL-ornithine

34.2 g. of 3-aminopiperidone-(2) hydrochloride are dissolved in 130 ml. of an aqueous solution containing 34% formaldehyde. The resulting solution, together with 10 g. of 10% palladium-deposited carbon, is placed in a 300 ml. autoclave into which hydrogen is pressed at an initial pressure of 120 kg./cm.<sup>2</sup>. With stirring the resulting mixture is maintained at room temperatures for 2 hours. After completion of the reaction, the catalyst is filtered off from the reaction mixture which is concentrated under reduced pressure, added with toluene and concentrated again. The residue is subjected to fractional distillation under reduced pressure to recover the fraction boiling at 127° C./mm. Hg. It is dissolved in 67 ml. of 4.5 N-HCl methanolic solution, and the resulted solution is concentrated and added with acetone thereby to form 45.4 g. of crude crystalline 3,3-dimethylamino-piperidone-(2) hydrochloride. Yield 85%. The crude crystals are dissolved in 23 ml. of methanol and added with 68 ml. of acetone. After standing the resulting mixture overnight, crystals are separated. Additionally 90 ml. of acetone are added to obtain a further crop of separated crystals. Yield 37.7 g. M.P. 202–204° C. (decomp., uncorrected). Elementary analysis is as follows:

Calcd. for  $C_7H_{15}N_2OCl$ : C, 47.05%; H, 8.46%; N, 15.68%. Found: C, 47.22%; H, 8.67%; N, 15.43%.

The thus obtained 3,3-dimethylamino-piperidone-(2) hydrochloride (8.9 g.) is heated at reflux for 3 hours with 50 ml. of an aqueous solution containing 6 g. of sodium hydroxide. The resulting aqueous solution is neutralized with 8.3 ml. of 6 N hydrochloride acid and then poured into 35 ml. of an aqueous solution containing 6.3 g. of cupric sulfate pentahydrate. The insoluble matters formed are taken away by filtration and the mother liquor is concentrated to have 50 ml. of an aqueous solution containing the copper salt of  $N^a,N^a$ -dimethyl-DL-ornithine. The aqueous solution is brought into reaction with lauroyl chloride and the resulted reaction mixture is treated with hydrogen sulfide for 60 minutes. The reaction mixture is filtered and the filtrate is concentrated under vacuum to obtain 10.3 g. of crude crystalline  $N^a,N^a$ -dimethyl- $N^e$ -lauroyl-DL-ornithine. Yield 60% based on 3,3-dimethylamino-piperidone-(2) hydrochloride. The crude crystalline product is dissolved in 4 times volume of ethanol and treated with active carbon. On adding 1.5 times volume of ether to the resulted solution, 9.1 g. pure desired product are obtained, M.P. 159–161° C. (uncorrected). Elementary analysis is given below:

Calcd. for  $C_{19}H_{38}N_2O_3$ : C, 66.62%; H, 11.18%; N, 8.18%. Found: C, 66.13%; H, 11.03%; N, 8.02%.

$N^a,N^a$ -dimethyl- $N^e$ -stearoyl-DL-ornithine

7.5 g. of  $N^a,N^a$ -dimethyl-DL-ornithine are dissolved in 100 ml. of an aqueous solution containing 10 g. of cupric acetate monohydrate. The resulting solution is concentrated and the separated crystalline mass is recrystallized from water. The copper salt of  $N^a,N^a$ -dimethyl-DL-ornithine is dissolved in 100 ml. of water. To the resulting solution, 100 ml. of ethyl ether is poured to form an upper layer. To the mixture with stirring and ice-cooling (0–5° C.) are added dropwise for 20 minutes 7 g. of stearoyl chloride dissolved in 50 ml. of ethyl ether and a normal sodium hydroxide solution sufficient to provide 1.1 moles of NaOH per mole of stearoyl chloride. Stirring is continued for additional two hours. The formed copper salt of  $N^a,N^a$ -dimethyl- $N^e$ -stearoyl-DL-ornithine precipitates as crystals which are collected by filtration. Yield 15 g. (70% on theoretical basis). The crude crystals are recrystallized from the small amount of ethanol to obtain 10 g. of the pure product.

5.0 grams of the pure copper salt are dissolved in 200 ml. of ethanol. Into the resulted solution, with stirring,

hydrogen sulfide gas is passed for 60 minutes. The reaction mixture is filtered and the filtrate is concentrated under reduced pressure to obtain 40 g. of crude crystalline  $N^a,N^a$ -dimethyl- $N^e$ -stearoyl-DL-ornithine. Yield 87%. The crude product is dissolved in 10 times amount by volume of ethanol and the resulted solution is treated with active carbon. After standing the filtrate overnight at 5° C., 2.0 g. of the pure product is obtained, which has a melting point of 154–156° C. (uncorrected). Elementary analysis of the product is as follows:

Calcd. for  $C_{25}H_{50}N_2O_3$ : C, 69.67%; H, 11.74%; N, 6.57%. Found: C, 70.37%; H, 11.81%; N, 6.37%.

$N^a,N^a$ -dimethyl- $N^e$ -myristoyl-DL-ornithine

7.5 g. of  $N^a,N^a$ -dimethyl-DL-ornithine are dissolved in 100 ml. of an aqueous solution containing 10 g. of cupric acetate monohydrate. The resulting solution is concentrated to have separated crystals which are purified by repeated recrystallization from water. The formed copper salt of  $N^a,N^a$ -dimethyl-DL-ornithine is reacted with myristoyl chloride in amount of 1.1 moles per mole of said copper salt, and then the resulted reaction product is treated with hydrogen sulfide in the same manner as in the preceding example, thereby to remove the copper. 8.0 g. of crude crystalline  $N^a,N^a$ -dimethyl- $N^e$ -myristoyl-DL-ornithine are obtained. Yield 46%. The crude product is dissolved in ethanol and the resulting solution is concentrated in vacuo thereby to obtain 40 g. of the pure product having a melting point of 120–125° C. (uncorrected). Elementary analysis is given below:

Calcd. for  $C_{21}H_{42}N_2O_3$ : C, 68.06%; H, 11.42%; N, 7.56%. Found: 67.50%; H, 11.61%; N, 6.89%.

$N^a,N^a$ -dimethyl- $N^e$ -lauroyl-DL-lysine

5.0 g. of  $N^a,N^a$ -dimethyl-DL-lysine are dissolved in methanol saturated with HCl. The resulting solution is heated under reflux and then concentrated under reduced pressure. The concentrated mass obtained is dissolved in chloroform and then added with 3.7 ml. of triethylamine and 5.7 g. of lauroyl chloride. After stirring, the resulted mixture is allowed to stand overnight at room temperature. The resulting reaction mixture is concentrated. The residue is dissolved in 75 ml. of methanol and added with 24 ml. of 2 N NaOH aq. The mixture is stirred at room temperature for one hour. The mixture is then neutralized with 12 ml. of 4 N HCl and concentrated under reduced pressure. The residual mass is added with a small quantity of ethanol and concentrated again under reduced pressure, thereby to remove water. The resulting water-free residue is dissolved in 20 ml. of hot ethanol. Undissolved sodium chloride is separated by filtration. After standing the filtrate in an ice box overnight, 2.8 g. of crude crystalline  $N^a,N^a$ -dimethyl- $N^e$ -lauroyl-DL-lysine are obtained. Yield 30.2% based on  $N^a,N^a$ -dimethyl-DL-lysine hydrochloride. The crude product is dissolved in 8.4 ml. of hot ethanol. The resulted solution is treated active carbon and then added with 10 ml. of ether. 6.6 g. of pure product as obtained, which has a melting point of 160–162° C. (uncorrected). Elementary analysis of this product is as follows:

Calcd. for  $C_{20}H_{40}N_2O_3$ : C, 67.37%; H, 11.31%; N, 7.86%. Found: C, 67.15%; H, 11.46%; N, 7.83%.

In carrying out the present invention in effect, a compound of the present invention is prepared as a solution (for example, 2% solution) dissolved in water or a water-miscible solvent, e.g. methanol, ethanol, acetone, etc., which solution is then added to a coating liquid. An amount of 1 to 50 ml. of 2% solution per 100 grams of the coating liquid usually is satisfactory. Any other known surface active agent may be used in combination with the coating aid of the present invention. In either case, the optimum amount of the coating aid used should be determined within the above-specified range, depending on the surfacial activity of the coating liquid, the contact

angle against the support or the required mobility or anti-static activity.

In the typical embodiment of the present invention, incorporation of a coating aid of the invention into a photographic emulsion can be made in the manner heretofore known per se in the art. For example, the coating aid can be added to the emulsion at any time just before, during or after the second ripening of the said emulsion. This photographic emulsion may be such that is sensitized by way of gold-, sulfur- or other chemical sensitization, for example, using polyalkylene oxide or optical sensitization. Further it may contain an azaindene stabilizer, a hardener, or a color former, if color film is to be prepared.

dimethyl - N<sup>a</sup> - lauroyl-DL-ornithine and N<sup>a</sup>,N<sup>a</sup>-dimethyl - N<sup>c</sup> - lauroyl-DL-lysine, are prepared as 3% aqueous solutions. The respective solutions are added at the amount of 6 ml. to each of three portions of the above-divided emulsion. To the remaining 100 g.-portions, 6 ml. of an aqueous solution of 3% saponine is added for comparison. The resulting mixtures are coated respectively to the subbed surfaces of cellulose triacetate film bases by dipping method.

On these cellulose triacetate films, the protective layers are provided by applying thereto 2% gelatine solution to which the above-used coating aids have been added correspondingly at the amount of 6 ml./100 g. of the gelatine solution. The results are set forth in the following tables.

TABLE 2

| Compound           | Coating                       | Notch at the periphery of coating | Number of coments per 1.0 m. <sup>2</sup> | Relative speed | Fog  |
|--------------------|-------------------------------|-----------------------------------|-------------------------------------------|----------------|------|
| II                 | Practically uniform           | None                              | 0                                         | 105            | 0.02 |
| III                | do                            | do                                | 1                                         | 100            | 0.03 |
| V                  | do                            | do                                | 0                                         | 102            | 0.02 |
| Saponine (control) | Unevenness appeared at random | do                                | 2                                         | 100            | 0.02 |

The following examples describe certain ways in which the principle of the invention has been applied, but are not to be construed as limiting its scope.

## EXAMPLE 1

N<sup>a</sup>,N<sup>a</sup>-dimethyl-N<sup>b</sup>-stearoyl-DL-ornithine (I), N<sup>a</sup>,N<sup>a</sup>-dimethyl-N<sup>c</sup>-palmitoyl-DL-lysine (IV) and N<sup>a</sup>,N<sup>a</sup>-dimethyl-N<sup>b</sup>-oleyl-DL-lysine (X) are prepared as 3% aqueous solutions, respectively. These aqueous solutions are individually added in their respective amount of 6 ml. to 100 g. of a high speed negative, photographic silver iodobromide emulsion. Each of the thus obtained emulsions is coated onto the subbed surface of cellulose triacetate film by means of double rollers. 100 g. of 2% gelatine solution are added with 6 ml. of each one of the above-named compounds (I), (IV) and (X). The gelatine solutions of the three kinds thus prepared are applied as protective layer onto the emulsion-coated surfaces of the above-said cellulose triacetate film bases, respectively.

For comparison, 6 ml. of an aqueous solution containing 2% sodium isoamyldecyldulfosuccinate (control) are added to 100 g. of the above-said photographic emulsion, which is then coated on the subbed surface of cellulose triacetate film. 2% gelatine emulsion to which the aqueous solution containing the control compound have been added at the amount of 6 ml. per 100 gram is placed as protective layer on the emulsion-coated surface of the above-said cellulose triacetate film.

The results are set forth in the following table.

TABLE 1

| Compound | Coating property                                 | Relative speed | Fog  | Gamma |
|----------|--------------------------------------------------|----------------|------|-------|
| I        | Neither unevenness nor repellency observed.      | 111            | 0.02 | 0.74  |
| IV       | do                                               | 107            | 0.02 | 0.77  |
| X        | do                                               | 108            | 0.02 | 0.71  |
| Control  | Unevenness in coating at random places observed. | 110            | 0.02 | 0.72  |

As shown in the above data, the compounds (I), (IV) and (X) of the invention serve to provide uniform coating without an adverse effect on the photographic properties of the resulting film.

## EXAMPLE 2

400 grams of a high speed photographic silver iodobromide emulsion is divided to four equal portions. The above-indicated compounds (II), (III) and (V), i.e. N<sup>a</sup>,N<sup>a</sup> - dimethyl - N<sup>b</sup> - myristoyl-DL-ornithine, N<sup>a</sup>,N<sup>a</sup> -

TABLE 3

| Compound           | Static electricity by separation at 20° C. and 40% R.H. (Coul- <sup>-12</sup> /7.07 cm. <sup>2</sup> ) | Specific surface resistance at 20° C. and 30% RH (ω) | Surface tension at 30° C. (dyne/cm.) | Contact angle at 40° C. (°) |
|--------------------|--------------------------------------------------------------------------------------------------------|------------------------------------------------------|--------------------------------------|-----------------------------|
| II                 | 67                                                                                                     | 9.4×10 <sup>15</sup>                                 | 36.2                                 | 32.6                        |
| III                | 25                                                                                                     | 9.9×10 <sup>15</sup>                                 | 35.8                                 | 32.0                        |
| V                  | 29                                                                                                     | 10.5×10 <sup>15</sup>                                | 34.5                                 | 32.3                        |
| Saponine (control) | 101                                                                                                    | 12.5×10 <sup>17</sup>                                | 43.4                                 | 45.4                        |

The above data indicate that coating aids of the present invention are comparable to saponine which is a relatively satisfactory coating aid known in the art. It is found that the coating aids of the invention are capable of providing uniform coating without an adverse effect on the photographic properties of the resulting films.

## EXAMPLE 3

To 100 grams of a silver chlorobromide emulsion for photographic papers, 1 ml. of an aqueous solution of 4% sodium isoamyldecyldulfosuccinate is added. The resulting mixture is coated on a baryta paper by dipping air-doctor method.

Separately, an aqueous solution containing 2% gelatine is prepared and divided to four equal portions. One of these portions is added with the said succinate aqueous solution at the amount of 0.5 ml. per 100 grams of the gelatine solution. The other three 100 g.-portions of the 2% gelatine solution are added with 3 ml. of an aqueous solution containing the specified compound, i.e. N<sup>a</sup>, N<sup>a</sup>-dimethyl - N<sup>b</sup> - palmitoyl-DL-lysine (IV), N<sup>b</sup>-palmitoyl-N<sup>a</sup>,N<sup>a</sup> - dimethyl-L-lysine (VII) or N<sup>a</sup>-palmitoyl-N<sup>a</sup>,N<sup>a</sup> - dimethyl-L-lysine methyl ester hydrochloride (VIII). The thus prepared coating liquids are used to provide protective layers on the emulsion-coated surface of the above papers.

Without causing any adverse effect on the quality of the photographic papers, uniform coating in double layers is obtained as indicated in the following table:

TABLE 4

| Compound: | Coating            | Number of coments per 1.0 m. <sup>2</sup> |
|-----------|--------------------|-------------------------------------------|
| IV        | Practically none   | 0                                         |
| VII       | do                 | 1                                         |
| VIII      | do                 | 0                                         |
| Control   | Appeared at random | 13                                        |

What is claimed is:

1. A photographic coating composition comprising a gelatine binder and, as a coating aid, an effective amount of a compound of the formula



5

wherein either X or Y is a lower dialkyl amino group of the formula



wherein R<sub>1</sub> and R<sub>2</sub> are lower alkyl groups and the other is an amido group of the formula —NHR<sub>3</sub> wherein R<sub>3</sub> is an acyl group of 6 to 18 carbon atoms; M is hydrogen or a lower alkyl group; and n is an integer from 2 to 4 inclusive.

2. A photographic coating composition as claimed in claim 1, wherein said compound is present in one or more layers selected from photo-sensitive layer, backing layer, protective layer, anti-halation layer and subbing layer.

3. A photographic coating composition as claimed in claim 1, wherein said compound is used in combination with a surface active agent.

4. A light-sensitive photographic silver halide emulsion comprising a gelatine binder and, as a coating aid, an effective amount of a compound of the formula



10

wherein either X or Y is a lower dialkyl amino group of the formula



8

10 wherein R<sub>1</sub> and R<sub>2</sub> are lower alkyl groups and the other is an amido group of the formula —NHR<sub>3</sub> wherein R<sub>3</sub> is an acyl group of 6 to 18 carbon atoms; M is hydrogen or a lower alkyl group; and n is an integer from 2 to 4 inclusive.

15 5. The emulsion as claimed in claim 4, further comprising a sulfur-, gold-, reductive or polyalkylene oxide sensitizer.

6. The emulsion as claimed in claim 4, further comprising an optical sensitizer.

20 7. The emulsion as claimed in claim 4, further comprising a color former.

#### References Cited

##### UNITED STATES PATENTS

25 2,240,471 4/1941 Swan ----- 96—94  
3,133,816 5/1964 Ben-Ezra ----- 96—94  
3,306,749 2/1967 Knox et al. ----- 96—94

30 NORMAN G. TORCHIN, Primary Examiner

M. F. KELLEY, Assistant Examiner

U.S. Cl. X.R.

106—125